

# UNITED STATES PATENT OFFICE.

THOMAS ALEX. DRAKE, OF JERSEY CITY, NEW JERSEY.

## LEATHER-DRESSING.

994,446.

Specification of Letters Patent.

Patented June 6, 1911.

No Drawing.

Application filed April 23, 1910. Serial No. 557,274.

To all whom it may concern:

Be it known that I, THOMAS A. DRAKE, citizen of the United States, residing at Jersey City, in the county of Hudson and State 5 of New Jersey, have invented certain new and useful Improvements in Leather-Dressings, of which the following is a specification.

This invention relates to improvements in 10 leather dressings and embraces the preparation of a compound capable of improving the finish of power belts or for waterproofing leather.

One form of the invention consists in 15 uniting the following elements or ingredients:

|                    |           |
|--------------------|-----------|
| Boiled linseed oil | 8 ounces. |
| Mutton tallow      | 8 ounces. |
| Yellow beeswax     | 8 ounces. |
| 20 Paraffin oil    | 8 ounces. |
| Common rosin       | 4 ounces. |

The above elements are placed in a water 25 and air tight vessel and steam cooked until thoroughly dissolved and united. This preparation forms a soft paste and serves to waterproof leather.

Another form of the invention consists of 30 the following preparation:

|                    |           |
|--------------------|-----------|
| Beeswax            | 2 ounces. |
| Boiled linseed oil | 6 ounces. |
| Paraffin oil       | 6 ounces. |
| Gum thus           | 7 ounces. |
| 35 Lard oil        | 6 ounces. |
| Castor oil         | 6 ounces. |
| Menhaden oil       | 6 ounces. |

The above elements are placed in a water 40 and air tight vessel and fused by steam.

The compound is useful for belt dressing.

Another form of the invention consists of 45 the following elements:

|              |           |
|--------------|-----------|
| Gum thus     | 8 ounces. |
| Lard oil     | 4 ounces. |
| Castor oil   | 4 ounces. |
| Menhaden oil | 4 ounces. |
| Paraffin oil | 4 ounces. |

|                    |           |    |
|--------------------|-----------|----|
| Beeswax            | 8 ounces. | 50 |
| Boiled linseed oil | 4 ounces. |    |
| Common rosin       | 8 ounces. |    |
| Petrolatum         | 3 ounces. |    |
| Beef tallow        | 3 ounces. |    |

The above elements are placed in a water 55 and air tight vessel and fused by steam. The compound thus formed is especially useful for oil soaked belts.

The improved compound is particularly 60 useful in improving the operating surfaces of power belts so that they will not slip; the ingredients, when applied thereto, giving the same a gripping surface.

Certain of the ingredients of the above 65 formula may be left out in order to make the compound more suitable for belts under certain conditions, or the proportions may be changed in order to make a compound of a suitable consistency; either oil, paste, or soap, or certain ingredients in the former 70 formula may be substituted for certain ingredients in this formula, to accomplish the same result, in fact the formulas may be changed in various ways without departing from the spirit of the invention, but 75

What I claim as new and desire to secure 80 by Letters Patent is—

1. A leather dressing comprising gum thus, lard oil, castor oil, menhaden oil, paraffin oil, beeswax and linseed oil, united by 85 heat.
2. A leather dressing containing gum thus and menhaden oil.

3. A leather dressing containing gum thus, menhaden oil and suitable oils, united by 85 heat.

4. A leather dressing containing suitable oils, waxes, petrolatum, menhaden oil and gum thus.

In testimony whereof I affix my signature 90 in presence of two witnesses.

THOMAS ALEX. DRAKE.

Witnesses:

ANNIE MARIA DRAKE,  
MARY M. DRAKE.